



US005484681A

# United States Patent

[19]

Cunningham et al.

[11] Patent Number: 5,484,681

[45] Date of Patent: Jan. 16, 1996

[54] CONDUCTIVE COMPOSITE PARTICLES  
AND PROCESSES FOR THE PREPARATION  
THEREOF

[75] Inventors: **Michael F. Cunningham**, Georgetown;  
**Hadi K. Mahabadi**, Toronto, both of  
Canada; **Thomas W. Smith**, Penfield;  
**John A. Creatura**, Ontario, both of  
N.Y.

[73] Assignee: **Xerox Corporation**, Stamford, Conn.

[21] Appl. No.: **331,469**

[22] Filed: **Oct. 31, 1994**

[51] Int. Cl.<sup>6</sup> ..... **G03G 9/113**

[52] U.S. Cl. ..... **430/137; 430/108**

[58] Field of Search ..... **430/108, 137**

[56] References Cited

U.S. PATENT DOCUMENTS

|           |         |              |         |
|-----------|---------|--------------|---------|
| 3,243,419 | 3/1966  | Ingram       | .       |
| 3,505,434 | 4/1966  | Battaerd     | 264/15  |
| 4,562,136 | 12/1985 | Inoue et al. | 430/107 |
| 4,590,141 | 5/1986  | Aoki et al.  | 430/108 |
| 4,833,060 | 5/1989  | Nair et al.  | 430/137 |

4,912,005 3/1990 Goodman et al. .... 430/108  
5,043,404 8/1991 Mahabadi et al. .... 526/194  
5,236,629 8/1993 Mahabadi et al. .... 252/511  
5,330,874 7/1994 Mahabadi et al. .... 430/108 X

Primary Examiner—Roland Martin  
Attorney, Agent, or Firm—E. O. Palazzo

[57] ABSTRACT

A process for the preparation of conductive submicron polymeric particles which comprises mixing at least one monomer with a polymerization initiator, a crosslinking component, and a chain transfer component; adding thereto an AB type block copolymer; effecting bulk polymerization until from about 10 to about 50 weight percent of the monomer has been polymerized; terminating polymerization by cooling the partially polymerized monomer; adding thereto from about 1 to about 50 weight percent of a conductive filler, or conductive fillers, followed by mixing thereof; dispersing the aforementioned mixture of conductive filler or fillers, and partially polymerized product in water containing a stabilizing component to obtain a suspension of particles with an average diameter of from about 0.05 to about 1 micron in water; polymerizing the resulting suspension by heating; and subsequently optionally washing and drying the product.

5 Claims, No Drawings

**CONDUCTIVE COMPOSITE PARTICLES  
AND PROCESSES FOR THE PREPARATION  
THEREOF**

**BACKGROUND OF THE INVENTION**

This invention is generally directed to submicron conductive composite particles and processes for the preparation thereof, and more specifically, the present invention relates to submicron, about 0.05 to about 0.99 in embodiments, conductive polymeric composite particles, each comprising a polymer, a conductive filler distributed evenly throughout the polymer matrix, and an AB block copolymer comprised of one block compatible with the polymer matrix, and a second block of a hydrophilic polymer, and with desirable charging properties residing on the copolymer surface that can enable either positive or negative triboelectric toner charge enhancement of from about 5 to about 25 microcou-  
lombs per gram. The present invention also relates to processes for the preparation of polymeric composite particles. In embodiments, the present invention comprises adding to the polymer base resin selected an AB block copolymer, such as a copolymer of polystyrene-b-polyacrylic acid, to enhance the negative tribo driving characteristics thereof, and such as polystyrene-b-polyoxyethylene copolymer to enhance the positive tribo driving characteristics thereof. In embodiments, the process of the present invention comprises the preparation of submicron conductive composite particles containing AB block copolymers and carbon black. In one embodiment, the process of the present invention comprises the preparation of conductive submicron polymeric particles containing a conductive filler distributed substantially throughout the polymer matrix of the particles and an AB block copolymer to enhance tribo charging, and which particles can be selected as carrier powder coatings. In another embodiment, the process of the present invention comprises the preparation of conductive polymeric composite particles with an average particle size diameter of from between about 0.05 micron to about 1 micron. The conductivity of the generated submicron polymeric composite particles can be modified by, for example, varying the weight percent of conductive filler component present in effective amounts of, for example, from between about 1 weight percent to about 50 weight percent, and also by varying the composition of the conductive filler component. Thus, conductive submicron polymeric composite particles with a conductivity of from between about  $10^{-10}$  (ohm-cm) $^{-1}$  to about  $10^{-4}$  (ohm-cm) $^{-1}$  can be prepared. In one process embodiment, the particles with average volume diameters of about 0.05 to about 1 micron are comprised of polymer, a conductive filler distributed evenly throughout the polymer matrix of the composite product or toner and an AB block copolymer, and which product can be obtained by a semisuspension polymerization method as illustrated in U.S. Pat. No. 5,043,404, the disclosure of which is totally incorporated herein by reference. In the aforementioned semisuspension polymerization processes, a mixture of monomer or comonomers, a polymerization initiator, a crosslinking component and a chain transfer component are bulk polymerized until partial polymerization is accomplished, for example. In one specific embodiment of the present invention, from about 10 to about 50 percent of monomer or comonomers are converted to polymer, thereafter the resulting partially polymerized monomer, or comonomers is cooled to cease bulk polymerization and to the cooled mixture of polymerized monomer, or comonomers is added a conductive filler, followed by mixing, using,

for example, a high shear mixer until a homogeneous mixer, or organic phase is obtained. Subsequently, the resulting organic phase is dispersed in water containing a stabilizing component with, for example, a high shear mixer; then the resulting suspension is transferred to a reactor and completely polymerized; the content of polymerization reactor is then cooled; followed preferably by washing and drying the polymer product. Also, there is needed a simple method whereby the triboelectric charge of the coated xerographic carrier can be enhanced in either a positive or negative direction, and this is accomplished in accordance with the present invention by the addition of certain AB block copolymers to the polymer composite particle. This process using the block copolymer provides considerably enhanced process latitude by enabling materials with different triboelectric behavior to be produced using the same polymer matrix with a small amount of block copolymer, rather than having to design and develop an entirely new polymer matrix.

Metals such as carrier cores are conductive or semiconductive materials, and the polymeric materials used to coat the surface of metals are usually insulating. Therefore, carrier particles coated completely with polymer or a mixture of polymers can lose their conductivity and become insulating. Although this is desired for some applications, for conductive magnetic brush systems (CMB) the carrier particles should be conductive. Since the carrier polymer coating can be utilized to control carrier tribo, a conductive carrier coating is needed to design carriers with the desired conductivity and triboelectrical properties. Conductive polymers can be very costly, and are not believed to be suitable for preparing low cost carrier components, for example less than \$5/pound, thus a conductive polymer composite comprising a low cost polymer and a conductive filler, such as conductive carbon black, is considered a more suitable alternative.

A polymer composite coating of metal materials, such as carrier beads, is known and can be obtained by two general approaches, solution and powder coating. Solution coating of carriers using a polymer composite solution comprised of a polymer, a conductive filler and solvent can be utilized to prepare conductive carrier, however, trapping of solvent in the solution coating adversely interferes with the use of coated materials, for example the residual solvent trapped in the carrier coating reduces the carrier life, and the release of solvent in the developer housing can cause other problems related to harmful effects of absorbed solvent to various copying machine parts and toxicity of solvent. Moreover, the solvent recovery operation involved in the solution coating processes is costly and can be hazardous. The powder coating of metal surfaces can eliminate the need for solvent, and therefore, many of the problems associated with solution coating; however, such processes require polymer powder with very small size, for example less than one micron in many situations. Although several polymer powders with desired particle size are available for carrier powder coating, submicron polymer composite particles containing conductive filler to prepare conductive coated carriers that maintain their triboelectrical characteristics for extended time periods exceeding, for example, 200,000 images are not believed to be available. Therefore, there is a need for conductive submicron polymeric composite particles, each containing a conductive filler distributed evenly throughout particles, and a process for preparing them, and for a simple method to be able to tailor the tribocharging characteristics of carrier particles.

The preparation of polymeric particles for powder coatings can be accomplished primarily by three methods,

namely grinding or attrition, precipitation and in situ particle polymerization. Grinding or attrition, especially fluid energy milling, of large polymeric particles or polymeric composite particles containing fillers to the size needed for powder coating, for example less than one micron, is often not desirable both from an economic and functional viewpoint. These materials are difficult to grind, and therefore, grinding or attrition of the required materials for coating with present milling equipment is very costly due to very low processing yield, for example in the range of 5 to 10 weight percent. Precipitation process can also be used to prepare polymeric/polymeric composite particles. In one approach, the polymer solution is heated to above its melting temperature and then cooled to form particles. In another process, the polymer solution is precipitated using a nonsolvent or the polymer solution is spray dried to obtain polymeric/polymeric composite particles. With all these precipitation processes, it has been difficult to achieve low cost and clean, that is, for example, with no or substantially no impurities such as solvents or precipitants in the resulting polymer particles. It is also difficult to obtain particles with small particle size and narrow particle size distribution. It is also difficult to control filler distribution throughout each particle's polymer matrix. In the in situ particle polymerization process, polymer particles are prepared by using suspension dispersion, emulsion and semisuspension polymerization. Suspension polymerization can be utilized to prepare polymer particles and polymeric composite particles containing, for example, a conductive filler. However, this process does not usually, for example, enable particles with a size less than five microns. Although emulsion and dispersion polymerization can be utilized to prepare polymeric particles of small size, for example less than one micron, these processes wherein particle formation is achieved by nucleation and growth do not readily enable synthesis of particles containing fillers such as conductive fillers. Conductive fillers, such as carbon blacks, are free radical polymerization inhibitors primarily reducing the rate of polymerization. Moreover, inclusion of fillers to obtain particles with evenly distributed fillers is not believed achievable with the prior art processes mentioned herein.

There is disclosed in U.S. Pat. No. 4,908,665 a developing roller or developer carrier comprised of a core shaft, a rubber layer and a resin coating layer on the surface of the rubber containing conductive fillers for a one component developer. It is indicated in the '665 patent that the conductive developing roller can eliminate variation of the image characteristics due to the absorption of moisture for one component development processes. This patent discloses a developing roller for one component developer and does not disclose, it is believed, the preparation of conductive carrier beads for dry two component developer. U.S. Pat. No. 4,590,141 discloses carrier particles for two component developer coated with a layer of silicon polymer using fluidized bed solution coating. U.S. Pat. No. 4,562,136 discloses a two component dry type developer which comprises carrier particles coated with a silicon resin containing a monoazo metal complex charging. The two component carriers described in the above two patents are insulating and are not believed to be conductive. There is disclosed in U.S. Pat. No. 4,912,005 a conductive carrier composition coated with a layer of resin containing a conductive particle by solution coating. Residual solvent trapped in the coated layer adversely effects the maintainability of the carrier electrical properties for an extended time period.

There is disclosed in U.S. Pat. No. 3,505,434 a process wherein particles for fluidized bed powder coating are

prepared by dispersing the polymer in a liquid which is heated to above the polymer melting point and stirred causing the polymer particles to form. The particles are then cooled below their melting point and recovered. However, this process does not, it is believed, for example, enable particles with a size of below 50 microns.

Also, the suspension polymerization of monomer is known for the formation of polymer/polymeric composite particles generally in a size range of about 200 microns and higher. The main advantage of suspension polymerization is that the product may easily be recovered, therefore, such a process is considered economical. However, it is very difficult by suspension polymerization to prepare very small particles as the monomer droplets tend to coalesce during the polymerization process, especially in the initial stage of polymerization where the droplets are very sticky. For example, there is disclosed in U.S. Pat. No. 3,243,419 a method of suspension polymerization wherein a suspending agent is generated during the suspension polymerization to aid in the coalescence of the particles. Also disclosed in U.S. Pat. No. 4,071,670 is a method of suspension polymerization wherein the monomer initiator mixture is dispersed in water containing stabilizer by a high shear homogenizer, followed by polymerization of suspended monomer droplets.

Further, disclosed in U.S. Pat. No. 4,835,084 is a method for preparing pigmented particles wherein high concentration of silica powder is used in the aqueous phase to prevent coalescence of the particles. There is also disclosed in U.S. Pat. No. 4,833,060 a process for the preparation of pigmented particles by dissolving polymer in monomer and dispersing in the aqueous phase containing silica powder to prevent coalescence of the particles. However, the silica powder used in both U.S. Pat. Nos. '084 and '060 should be removed using KOH, which is costly, and residual KOH and silica materials remaining on the surface affects the charging properties of particles. Moreover, the above patents do not disclose, it is believed, the preparation of submicron conductive particles. There is also disclosed in U.S. Pat. No. 3,954,898 a two step polymerization process for the preparation of a thermosetting finished powder. However, this process does not enable, it is believed, synthesis of particles with size less than 100 microns. Moreover, this patent does not teach the synthesis of submicron particles containing conductive fillers.

As a result of a patentability search in the aforementioned U.S. Pat. No. 5,043,404, the disclosure of which is totally incorporated herein by reference, there were located U.S. Pat. No. 4,486,559, which discloses the incorporation of a prepolymer into a monomer toner mix followed by emulsion polymerization; 4,680,200 and 4,702,988, which illustrate emulsion polymerization. It is known that submicron polymeric particles can be synthesized by emulsion polymerization. However, synthesis of submicron polymeric particles by emulsion polymerization requires a high concentration of emulsifier which remains in the final product and, it is believed, renders it humidity sensitive. Therefore, emulsion polymerization does not, it is believed, enable preparation of clean submicron polymeric particles which are insensitive to humidity. Moreover, in the emulsion polymerization, particle formation is controlled by diffusion of monomer from monomer droplet through a water phase into the growing particles. This mechanism, which is characteristic of emulsion polymerization, does not allow, it is believed, inclusion of conductive fillers in the polymeric particles. Furthermore, it is known that the addition of conductive fillers into emulsion, dispersion or suspension polymerization systems can cause severe inhibition which cancels or reduces the rate of polymerization significantly.

Disclosed in the aforementioned U.S. Pat. No. 5,043,404, the disclosure of which is totally incorporated herein by reference, is a semisuspension polymerization process for the preparation of small polymeric particles which are comprised of a mixture of monomer or comonomers, a polymerization initiator, a crosslinking component and a chain transfer component which are bulk polymerized until partial polymerization is accomplished. The resulting partially polymerized monomer or comonomers are dispersed in water containing a stabilizer component with, for example, a high shear mixer, then the resulting suspension polymerized, followed by washing and drying the submicron polymeric particles. However, U.S. Pat. No. 5,043,404 does not, it is believed, disclose submicron conductive polymeric particles containing conductive fillers.

U.S. Pat. No. 5,236,629 describes a process for the preparation of conductive submicron polymeric particles which comprises mixing at least one monomer with a polymerization initiator, a crosslinking component and a chain transfer component; effecting bulk polymerization until from about 10 to about 50 weight percent of the monomer has been polymerized; terminating polymerization by cooling the partially polymerized monomer; adding thereto from about 1 to about 50 weight percent of a conductive filler, or conductive fillers, followed by mixing thereof; dispersing the aforementioned mixture of conductive filler or fillers, and partially polymerized product in water containing a stabilizing component to obtain a suspension of particles with an average diameter of from about 0.05 to about 1 micron in water; polymerizing the resulting suspension by heating; and subsequently washing and drying the product. However, the triboelectric charge of the polymeric particle is primarily effected by the type of polymer selected for the matrix and to a lesser extent the particular conductive additive used. The tribocharge of the coated carrier cannot be easily varied. To vary the triboelectric charge of the coated carrier using the process described in the 5,236,629 patent, it is necessary to formulate an entirely new product, by for example using a different selection of monomers. There is currently no suitable effective means available to vary the triboelectric charge of a single material without developing a completely new material or blending that material with one or more additional polymers. Therefore, it would be an advantage to have a simple means of modifying the triboelectric charge to enable broader design latitude while being able to preserve the essential identity of an existing product and without having to develop or employ additional materials.

There thus remains a need for submicron conductive polymeric particles for which the triboelectric charge can be easily enhanced in either the positive or negative direction, and more specifically, conductive submicron polymeric particles containing conductive fillers distributed throughout each particle for which the triboelectric charge can be easily enhanced in either the positive or negative direction. Further, there is a need for a process to obtain conductive submicron polymer particles, each containing conductive fillers evenly distributed in the polymer and an AB block copolymer, and more specifically, there is a need for a semisuspension polymerization process for obtaining low cost clean and dry small, for example from about 0.05 to about 1 micron in average diameter as determined by a scanning electron microscope, polymeric particles containing from about 1 to about 50 weight percent of a conductive filler, such as carbon black, which is evenly distributed throughout the polymer matrix, and containing from about 1 to about 10 weight percent of an AB block copolymer.

The criteria for selection of the A and B blocks of the block copolymer are of importance to the process of the present invention. The A block polymer is to be non-water soluble (less than 1 weight percent solubility in water); the B block polymer is to be excellent water solubility (greater than about 5 percent). During the particle formation and subsequent suspension polymerization, there exists a thermodynamic driving force for the block copolymer to partition such that the hydrophobic A block remains in the particle interior while the hydrophilic B block migrates to the particle surface. However, the presence of the hydrophobic A block prevents migration of the B block out of the particle. Because of its location on the particle surface, a relatively small amount of B block will have a significant effect on overall triboelectric charging of the particle. Positive or negative charging can be enhanced by appropriate choice of the B block polymer, for example polyacrylic acid will enhance negative charging while polyethylene oxide will enhance positive charging.

The block copolymer can be prepared by any known means for preparing block copolymers, for example, such as ionic polymerization or group transfer polymerization, see the *Encyclopedia of Polymer Science and Engineering*, Volume 2, page 324, John Wiley and Sons, New York, 1984, the disclosure of which is totally incorporated herein by reference.

#### SUMMARY OF THE INVENTION

It is, therefore, an object of this invention to provide conductive submicron polymeric composite particles and processes thereof with many of the advantages illustrated herein.

In another object of the present invention there are provided conductive submicron polymeric composites comprised of a polymer and a conductive filler distributed evenly throughout the polymer matrix of the composite, and an AB block copolymer to enhance triboelectric charging in either a positive or negative charge direction and processes for the preparation thereof.

In yet another object of the present invention there are provided low cost, clean and dry conductive submicron polymeric composite particles comprised of from about 50 to about 99 weight percent of polymer and from about 1 to about 50 weight percent of conductive filler distributed throughout the polymer matrix of the composite as measured by TEM, and from about 1 to about 10 weight percent of an AB block copolymer that provides enhanced triboelectric charging properties, and processes for the preparation thereof.

Another object of the present invention resides in conductive submicron polymeric composite particles with a conductivity from about  $10^{-10}$  ( $\text{ohm}\cdot\text{cm}$ ) $^{-1}$  to about  $10^{-4}$  ( $\text{ohm}\cdot\text{cm}$ ) $^{-1}$  and processes for the preparation thereof.

Another object of the present invention resides in conductive submicron polymeric composite particles with an average volume particle diameter size of from about 0.05 micron to about 1 micron.

In another object of the present invention there are provided conductive submicron polymeric composites, which can be selected for two component carrier powder coatings, and processes for preparing such particles.

In another object of the present invention there are provided simple processes for the formation of small conductive polymeric particles, and more specifically, submi-

cron size conductive polymeric particles with preselected tailored triboelectric charging behavior.

Also, in another object of the present invention there are provided simple and economical processes for the formation of conductive submicron polymeric particles that can be selected as carrier coatings, reference U.S. Pat. Nos. 4,937,166 and 4,935,326, the disclosures of which are totally incorporated herein by reference.

Another object of the present invention resides in simple and economical semisuspension polymerization processes for the preparation of low cost, clean, and dry submicron conductive polymeric particles, and more specifically, submicron size conductive polymeric particles useful as carrier powder coatings.

Additionally, in another object of the present invention there are provided as a result of the enhanced degree of control and flexibility processes for the preparation of polymeric particles containing a conductive filler, or fillers with improved flow and fusing properties, and particles that can be selected for conductive carrier powder coating with a triboelectric charge in the range, for example, of from about -40 to about +40 microcoulombs per gram as determined by the known Faraday Cage process.

These and other objects of the present invention can be accomplished in embodiments by the provision of processes for the preparation of submicron conductive polymer particles, each containing conductive filler or fillers, distributed evenly throughout the polymer matrix of the particles and an AB block copolymer, referred to as semisuspension polymerization processes in which a mixture of monomer or comonomers, a polymerization initiator, an optional crosslinking component and an optional chain transfer component together with an AB block copolymer is bulk polymerized until partial polymerization is accomplished, for example from about 10 to about 50 percent of monomer or comonomers is converted to polymer. The bulk polymerization is then terminated by cooling the partially polymerized monomer or comonomers. To the cooled partially polymerized product there is then added a conductive filler, followed by mixing thereof with, for example, a high shear homogenizer, such as a Brinkman homogenizer to prepare a mixture, or organic phase. The viscosity of the organic phase can in embodiments be an important factor in controlling dispersion of the conductive filler in the particles, and which viscosity can be adjusted by the percentage of polymer in the mixture. The aforementioned partially polymerized product with filler is then dispersed in water containing a stabilizing component with, for example, a high shear mixer to permit the formation of a suspension containing small, less than 10 microns for example, particles therein, and thereafter, transferring the resulting suspension product to a reactor, followed by polymerization until complete conversion to the polymer product is achieved. The polymer product can then be cooled, washed and dried. More specifically, the process of the present invention is comprised of (1) mixing a monomer or comonomers with polymerization initiators, a crosslinking component and a chain transfer component; (2) adding an AB block copolymer such that the A block is compatible with the polymer matrix and the B block is a hydrophilic polymer that provides enhanced triboelectric charging in the desired positive or negative direction; and effecting bulk polymerization by increasing the temperature of the aforementioned mixture to from about 45° C. to about 120° C. until from about 10 to about 50 weight percent of monomer or comonomers has been polymerized; the molecular weight of polymer in the bulk or the percentage of polymer present in the mixture which affects the viscosity

of the partially polymerized monomer or comonomers can be an important factor in controlling conductive filler distribution in the particles; (3) cooling the partially polymerized monomer or comonomers and adding a conductive filler, followed by mixing thereof with, for example, a high shear homogenizer to form an organic phase; (4) dispersing the organic phase in from about 2 to about 5 times its volume of water containing from about 1 to about 5 weight percent of a stabilizing component to form a suspension with a particle size diameter of from about 0.05 micron to about 1 micron particles containing from about 1 to about 50 weight percent of a conductive filler, or conductive fillers using a high shear mixer; (5) transferring the resulting suspension to a reactor and polymerizing the suspension by increasing its temperature to from about 45° C. to about 120° C. to allow the complete conversion of monomer or comonomers to polymer; (6) cooling the product and washing the product with, for example, water and/or an alcohol like methanol; (7) separating polymer particles from the water/methanol by means of filtration or centrifugation; and (8) drying the polymeric particles.

One specific embodiment of the present invention comprises the preparation of polymeric particles, which comprises mixing at least one monomer with a polymerization initiator, a crosslinking component and a chain transfer component; adding an AB block copolymer; effecting bulk polymerization until from about 10 to about 50 weight percent of the monomer has been polymerized; adding a conductive filler thereto and mixing; dispersing the aforementioned product in water containing a stabilizing component to obtain a suspension of particles with an average diameter of from about 0.05 to about 1 micron in water; and polymerizing the resulting suspension. By at least one monomer is intended to include from about 2 to about 20 monomers, comonomers thereof, and the like. Throughout "from about to about" includes between the ranges provided.

The present invention is directed to the preparation of small conductive polymeric particles, that is with, for example, an average particle diameter in the range of from about 0.05 micron to about 1 micron, and preferably from about 0.1 to about 0.8 micron as measured by SEM containing 1 to about 50 percent and preferably 10 to 20 percent conductive filler distributed throughout the polymer matrix of particles, and with about 0.5 to 25 weight percent, and preferably from about 1 to 10 weight percent of an AB block copolymer, and which polymer particles have a number and weight average molecular weight of from between about 5,000 to about 500,000 and from between about 10,000 to about 2,000,000, respectively, in embodiments.

Further, the process of the present invention is directed to the preparation of conductive polymeric particles of average diameter of from about 0.1 micron to about 0.8 micron containing 10 to 20 weight percent of a conductive filter and 80 to 90 weight percent of a polymeric material. This polymeric material can be comprised of a linear and crosslinked portions with a number average molecular weight of the linear portion being from about 5,000 to about 50,000 and a weight average molecular weight of from about 100,000 to about 500,000 and from 0.1 to about 5 weight percent of a crosslinked portion, and a third portion which is an AB block copolymer with the number average molecular weight of the A block of the AB type block copolymer component being in the range of from about 500 to about 500,000 and more preferably from about 10,000 to about 100,000, and the number average molecular weight of the B block of the AB type block copolymer component being in the range from about 500 to about 1,000,000 and, more

preferably, from about 1,000 to about 50,000, and which polymer product is useful for carrier coatings. More specifically, the process of the present invention in embodiments is directed to the preparation of conductive polymeric particles of an average diameter in the range of between about 0.1 to about 0.8 micron with conductive filler distributed evenly throughout the resulting polymer matrix as measured by TEM with a linear portion having a number average molecular weight in the range of from about 5,000 to about 50,000, and a weight average molecular weight of from about 100,000 to about 500,000, and from about 0.1 to about 5 weight percent of a crosslinked portion, and about 1 to 10 weight percent of an AB block copolymer. This process as indicated herein comprises (1) mixing a monomer or comonomers with a polymerization initiator with the ratio of monomer or comonomers to initiator being from about 100/2 to about 100/20, a crosslinking component with the ratio of monomers or comonomers to crosslinking component being from about 100/0.1 to about 100/5, and a chain transfer component with the ratio of monomer or comonomers to the chain transfer component being from about 100/0.01 to about 100/1; (2) adding an AB block copolymer such that the A block is compatible with the polymer matrix and the B block is a hydrophilic polymer that provides enhanced triboelectric charging in the required positive or negative direction, the AB block is added with the ratio of monomer or monomers to AB block copolymer being from about 100/1 to about 100/25, and the ratio of the A block to the B block being from about 100/10 to about 10/100; (3) effecting bulk polymerization by increasing the temperature of the mixture to from about 45° C. to about 120° C. until from about 10 to about 50 weight percent of monomer or comonomers has been converted to polymer with a number average molecular weight of from 5,000 to about 50,000 and a weight average molecular weight of from about 10,000 to about 40,000, and thereafter, adding conductive filler thereto with the ratio of filler to polymer monomer mixture being from about 0.1 to about 0.2, followed by extensive mixing to prepare organic phase; (4) dispersing the resulting organic phase from about 2 to about 5 times its volume in water containing from about 1 to about 5 weight percent of a stabilizing component, preferably polyvinylalcohol having a weight average molecular weight of from about 1,000 to about 10,000 to form a suspension containing particles with a particle size diameter of from about 0.1 to about 0.8 micron by using high shear mixer; (5) transferring the resulting suspension to a reactor and polymerizing the suspension by increasing its temperature to from about 45° C. to about 120° C. to allow the complete conversion of monomer or comonomers to polymer; (6) washing the resulting product with equal volumes of methanol and/or water from about 3 to about 5 times; (7) separating polymeric particles from water/methanol by means of filtration or centrifugation; and (8) drying of the polymeric particles.

In an embodiment, the present invention is directed to a process for the preparation of conductive submicron polymeric particles, which comprises mixing at least one monomer with a polymerization initiator, a crosslinking component and a chain transfer component; adding an AB block copolymer with the A block being a polymer that is compatible with the polymeric particle matrix polymer and the B block being a hydrophilic polymer that provides the required enhanced charging; effecting bulk polymerization until from about 10 to about 50 weight percent of the monomer has been polymerized; terminating polymerization by cooling the partially polymerized monomer; adding thereto from about 1 to about 50 weight percent of a

conductive filler, or conductive fillers, followed by mixing thereof; dispersing the aforementioned mixture of conductive filler or fillers, and partially polymerized product in water containing a stabilizing component to obtain a suspension of particles with an average diameter of from about 0.05 to about 1 micron in water; polymerizing the resulting suspension by heating; and subsequently washing and drying the product.

Illustrative examples of monomer or comonomers preferably selected in an amount of, for example, from about 80 to about 99 weight percent include vinyl monomers comprised of styrene and its derivatives such as styrene,  $\alpha$ -methylstyrene, p-chlorostyrene, and the like; monocarboxylic acids and their derivatives such as acrylic acid, methyl acrylate, ethyl acrylate, butyl acrylate, dodecyl acrylate, octyl acrylate, phenyl acrylate, methacrylic acids, methyl methacrylate, ethyl methacrylate, butyl methacrylate, octyl methacrylate, acrylonitrile and acrylamide; dicarboxylic acids having a double bond and their derivatives such as maleic acid, monobutyl maleate, dibutylmaleate; vinyl esters such as vinyl chloride, vinyl acetate and vinyl benzoate; vinyl ketones such as vinyl methyl ketone and vinyl ether ketone; and vinyl ethyl ether and vinyl isobutyl ether; vinyl naphthalene; unsaturated mono-olefins such as isobutylene, and the like; vinylidene halides such as vinylidene chloride and the like; N-vinyl compounds such as N-vinyl pyrrole and fluorinated monomers such as pentafluoro styrene, allyl pentafluorobenzene and the like; and mixtures thereof.

Illustrative examples of polymerization initiators selected in an amount of, for example, from about 0.1 to about 20 weight percent of monomer include azo compounds such as 2,2'-azodimethylvaleronitrile, 2,2'-azoisobutyronitrile, azobiscyclohexanenitrile, 2-methylbutronitrile, and the like, and peroxide such as benzoyl peroxide, lauryl peroxide, 1-1-(t-butylperoxy)-3,3,5-trimethylcyclohexane, n-butyl-4, 4-di-(t-butylperoxy)valerate, dicumyl peroxide, and the like.

Crosslinkers selected for the process of the present invention are known and can be comprised of compounds having two or more polymerizable double bonds. Examples of such compounds include aromatic divinyl compounds such as divinylbenzene and divinylnaphthalene; carboxylic acid esters having two double bonds such as ethylene glycol diacrylate, ethylene glycol dimethylacrylate, and the like; divinyl compounds such as divinyl ether, divinyl sulfite, divinyl sulfone, and the like. Among these divinylbenzene is particularly useful. The crosslinking component is preferably present in an amount of from about 0.1 to about 5 parts by weight in 100 parts by weight of monomer or comonomers mixture.

Examples of conductive fillers present in effective amounts as illustrated herein, for example, include conductive carbon blacks such as acetylene black, available from Chevron Chemical, VULCAN BLACK™, BLACK PEARL L®, KEYTJEN BLACK EC600JD®, available from AK20, CONDUCTEX SC ULTRA™, available from Columbian-Chemical, metal oxides such as iron oxides,  $TiO_2$ ,  $SnO_2$  and metal powders such as iron powder.

Stabilizers selected in an amount of, for example, from about 0.1 to about 5 weight percent of water are selected from the group consisting of both nonionic and ionic water soluble polymeric stabilizers such as methyl cellulose, ethyl cellulose, hydroxypropyl cellulose, block copolymer such as PLURONIC E87™ from BASF, sodium salt of carboxyl methyl cellulose, polyacrylate acids, and their salts; polyvinyl alcohol, gelatins, starches, gums, alginates, zein and

casein, and the like; and barrier stabilizers such as tricalcium phosphate, talc, barium sulfate, and the like. Among these, polyvinyl alcohol with a weight average molecular weight of from about 1,000 to about 10,000 is particularly useful.

Chain transfer components selected, which primarily function to control molecular weight by inhibiting chain growth, include mercaptans such as laurylmercaptan, butylmercaptan, and the like, or halogenated carbons such as carbon tetrachloride or carbon tetrabromide, and the like. The chain transfer agent is preferably present in an amount of from about 0.01 to about 1 weight percent of monomer or comonomer mixture. Also, stabilizer present on the surface of the polymeric particles can be washed using an alcohol such as, for example, methanol, and the like, or water. Separation of washed particles from solution can be achieved by any classical separation technique such as filtration, centrifugation, and the like. Classical drying techniques such as vacuum drying, freeze drying, spray drying, fluid bed drying, and the like can be selected for drying of the polymeric particles.

Illustrative specific examples of polymer or copolymer products present in an amount of about 50 to about 99 weight percent containing, for example, both a linear and a crosslinked portion in which the ratio of crosslinked portion to linear portion is from about 0.001 to about 0.05, and the number and weight average molecular weight of the linear portion is from about 5,000 to about 500,000 and from about 10,000 to about 2,000,000, respectively, include vinyl polymers of polystyrene and its copolymers, polymethylmethacrylate and its copolymers, unsaturated polymers or copolymers such as styrene-butadiene copolymers, fluorinated polymers or copolymers such as poly(pentafluorostyrene) poly(pentafluorobenzene), and the like.

Illustrative specific examples of monomers used in forming the A block of the AB type block copolymer component include monomers that polymerize to polymers with low water solubility, less than 1, and preferably about 0.5 weight percent, for example, such as  $\alpha$ -methyl-styrene, p-chlorostyrene; vinyl ketones; vinyl naphthalene; unsaturated monoolefins; vinylidene halides; fluorinated vinyl compounds, methyl acrylate, ethyl acrylate, butyl acrylate, dodecyl acrylate, octyl acrylate, phenyl acrylate, methyl methacrylate, ethyl methacrylate, butyl methacrylate, octyl methacrylate, monobutyl maleate, dibutyl maleate; vinyl chloride, and vinyl benzoate; vinylidene chloride; pentafluoro styrene and allyl pentafluorobenzene.

Illustrative specific examples of monomers used in forming the B block of the AB type block copolymer component include monomers that polymerize to polymers with high water solubilities in excess of about 5, such as about 10 weight percent, such as acrylic acids, methacrylic acids, acrylamide, acrylonitrile, ethylene oxide, N-vinyl pyrrolidone, maleic acid, vinylsulfonic acid, styrenesulfonic acid, 2-acrylamido-2-methylpropanesulfonic acid, 3-vinylxylopropane-1-sulfonic acid, 2-methacryloyloxy ethanesulfonate, 3-methacryloyloxy-2-hydroxypropanesulfonate, 2-acrylamido-2-methyl propanesulfonate, 3-sulfo-2-hydroxypropyl methacrylate, vinylphosphonic acid, 4-vinylphenol, N-vinylsuccinimide acid; diallyldimethylammonium chloride, diallyldiethylammonium chloride, diethylaminoethyl methacrylate, dimethylaminoethyl methacrylate, methacryloyloxyethyl trimethylammonium sulfate, methacryloyloxyethyl trimethylammonium chloride, and 3-(methacrylamido)propyltrimethylammonium chloride.

The resulting polymer composite particles with, for example, fillers of the present invention can be selected as

carrier powder coatings, which carriers contain, for example, a steel or ferrite core, and can be admixed with toner compositions comprised of resin particles, pigment particles and optional additives such as charge control components, reference U.S. Pat. No. 4,560,635, the disclosure of which is totally incorporated herein by reference, enabling the formation of a developer composition useful in electrophotographic imaging processes.

The following Examples are being submitted to further define various species of the present invention. These Examples are intended to be illustrative only and are not intended to limit the scope of the present invention. Also, parts and percentages are by weight unless otherwise indicated.

#### EXAMPLE I

Methylmethacrylate monomer (200 grams) was added to 6 grams of 2,2'-azobis(2,4-dimethylvaleronitrile), 1.6 grams of benzoyl peroxide and 0.85 gram of divinyl benzene crosslinking agent, and mixed in a one liter flask using a mechanical stirrer. To this mixture were added 10 grams of the block copolymer polystyrene-b-polyethylene oxide. This block copolymer contained 40 weight percent of polystyrene and 60 weight percent of polyethylene oxide. The number average molecular weights of the polystyrene and polyethylene oxide blocks were 15,000 and 8,000, respectively. The mixture was bulk polymerized by heating to 45° C. until 12 weight percent of the monomer as measured by gravimetry was converted to polymer. The bulk polymerization was quenched by cooling, and then 30 grams of CONDUCTEX SC ULTRA® carbon black were added and the contents were mixed using a Brinkmann Polytron homogenizer to produce a homogeneous organic phase mixture. This organic phase was then poured into a container along with 650 grams of an aqueous solution of 4 weight percent of polyvinyl alcohol having a weight average molecular weight of 3,000, and the resulting mixture was then homogenized for 5 minutes to produce a microsuspension of polymeric particles containing carbon black in water. A quantity of 5.0 grams of potassium iodide was then added as an aqueous phase inhibitor. The resulting microsuspension was transferred to a 1 liter stainless steel reactor and the temperature was raised from 25° to 60° C. in 35 minutes where it was held for 2 hours; the temperature was then increased to 85° C. during a 2 hour period and held there for 1 hour, after which the suspension was cooled in 30 minutes to 25° C. When cooled to 25° C., the suspension polymerization was complete as measured using gas chromatography. The microsuspension product was then poured into 1 liter of methanol. The resulting diluted suspension was centrifuged. The resulting supernatant liquid comprised of the diluted polyvinyl alcohol was decanted, fresh methanol/water 50:50 ratio was added, and the resulting mixture was mixed for 1 to 2 minutes at 5,000 revolutions per minute. This washing procedure was again repeated with deionized water. After the final wash, the product was freeze dried to provide dry individual particles. Scanning electron microscope (SEM) photomicrographs of the dry product indicated that the average particle size of the polymer product was 0.7 micron. The glass transition temperature of 113° C. was measured by DSC. The polymer product conductivity was measured by melting one gram of product in the form of film, and using a conductivity meter, the results showed a conductivity of  $10^{-8}$  (ohm-cm) $^{-1}$ . 0.7 Gram of the resulting polymethyl methacrylate particles containing carbon black with block copolymer were mixed with 100 grams of an iron core

## 13

carrier with an average bead diameter of 90 microns in a Munson type mixer at room temperature. The coated materials were then fused on the surface of the carrier at 350° F. in a rotary kiln furnace. The product was sieved through a 177 micron screen to remove coarse materials. The coarse fraction was found to be about 0.1 weight percent. The sieved materials were scanned for surface coverage using SEM. The results evidenced 100 percent surface coverage of polymer. The functional evaluation of the resulting carrier in the Xerox Corporation 5100 two component development system indicated a triboelectric charge (tribo) of 41 microcoulombs per gram as determined by the Faraday Cage method.

## EXAMPLE II

Styrene monomer (200 grams) was added to 8 grams of 2,2'-azobis(2,4-dimethylvaleronitrile), 2.0 grams of benzoyl peroxide and 0.65 grams of divinyl benzene crosslinking agent, and mixed in a one liter flask using a mechanical stirrer. To this mixture were added 10 grams of a block copolymer of polystyrene-b-polyethylene oxide. This block copolymer contained 40 weight percent of polystyrene and 60 weight percent of polyethylene oxide. The number average molecular weights of the polystyrene and polyethylene oxide blocks were 15,000 and 8,000, respectively. The mixture was bulk polymerized by heating to 55° C. until 16 weight percent of the monomer as measured by gravimetry was converted to polymer. The bulk polymerization was quenched by cooling and then 30 grams of CONDUCTEX SC ULTRA® carbon black were added and the contents were mixed using a Brinkmann Polytron homogenizer. The resulting organic phase was then poured into a flask, along with 650 grams of an aqueous solution of 4 weight percent of polyvinyl alcohol having a weight average molecular weight of 3,000, and the resulting mixture was then homogenized for 5 minutes to produce a microsuspension of polymeric particles containing carbon black in water. A quantity of 5.0 grams of potassium iodide was then added as an aqueous phase inhibitor. The organic phase mixture was then polymerized by heating, reference Example I. The same carrier coating procedure as described in Example I was then repeated. The coated carrier had a tribo of 19.8 microcoulombs per gram.

## EXAMPLE III

The process of Example I was repeated except that the block copolymer selected was a polystyrene-b-polyacrylic acid block copolymer. This block copolymer contained 50 weight percent of polystyrene. The coated carrier had a tribocharge of 22.4 microcoulombs per gram.

## EXAMPLE IV

The process of Example II was repeated except that the block copolymer selected was a polystyrene-b-polyacrylic acid block copolymer. This block copolymer contained 50 weight percent of polystyrene. The coated carrier had a tribocharge of 3.3 microcoulombs per gram.

## EXAMPLE V

The process of Example I was repeated except that no block copolymer was selected. The coated carrier had a tribocharge of 29.8 microcoulombs per gram.

## 14

## EXAMPLE VI

The process of Example II was repeated except that no block copolymer was selected. The coated carrier had a tribocharge of 12.5 microcoulombs per gram.

## EXAMPLE VII

The process of Example I was repeated except that the block copolymer was a polystyrene-b-polymethylmethacrylate polymer comprised of 45 percent polystyrene. This material does not have a suitable B block as described herein in that polymethylmethacrylate is not sufficiently hydrophilic and hence will not diffuse to the particle surface. The coated carrier had a tribocharge of 29.1 microcoulombs per gram, which is the same charge resulting when no block copolymer is used (Example V).

## EXAMPLE VIII

The process of Example II was repeated except that the block copolymer was a polystyrene-b-polymethylmethacrylate polymer comprised of 45 percent polystyrene. This material does not have a suitable B block as polymethylmethacrylate is not sufficiently hydrophilic and hence will not diffuse to the particle surface. The coated carrier had a tribo charge of 12.9 microcoulombs per gram, which is the same charge resulting when no block copolymer is used (Example VI).

## EXAMPLE IX

The process of Example I was repeated except a mixture of styrene and methylmethacrylate with 20 weight percent of styrene and 90 weight percent of methylmethacrylate comonomer was used in place of the monomers of Example I. The resulting submicron polymeric particles and coated carrier possessed properties similar to that of Example I, and wherein the tribocharge of the coated carrier was 18 microcoulombs per gram.

## EXAMPLE X

The process of Example IV was repeated except styrene monomer was used. Submicron conductive particles and coated carrier with the same properties of Example IV except with a tribocharge of 5 microcoulombs per gram were obtained.

## EXAMPLE XI

The process of Example IV was repeated except a mixture of 20 weight percent of acrylic acid and 80 weight percent of styrene comonomer was used. There resulted submicron conductive particles and coated carrier thereof with the same properties as that of Example IV except with a carrier tribocharge of -10 microcoulombs per gram.

## EXAMPLE XII

The process of Example IV was repeated except pentfluorostyrene monomer was used. There resulted submicron conductive particles and xerographic coated carrier thereof with the same properties as that of Example IV except with a tribocharge of -25 microcoulombs per gram were obtained.

## 15

## EXAMPLE XIII

The process of Example IV was repeated except allyl pentafluorobenzene monomer was used in place of methyl-methacrylate monomer. There resulted submicron conductive particles and coated carrier thereof with the same properties as that of Example IV except with a tribocharge of -35 microcoulombs per gram were obtained.

Other modifications of the present invention may occur to those skilled in the art subsequent to a review of the present application. The aforementioned modifications, including equivalents thereof, are intended to be included within the scope of the present invention.

What is claimed is:

1. A process for the preparation of carrier particles which carrier particles consist of a core and a coating thereover, and wherein said coating is prepared by mixing at least one monomer with a polymerization initiator, a crosslinking component, and a chain transfer component; adding thereto an AB type block copolymer; effecting bulk polymerization until from about 10 to about 50 weight percent of the monomer has been polymerized; terminating polymerization by cooling the partially polymerized monomer; adding thereto from about 1 to about 50 weight percent of a conductive filler, or conductive fillers, followed by mixing thereof; dispersing the aforementioned mixture of conductive filler or fillers, and partially polymerized product in water containing a stabilizing component to obtain a suspension of particles with an average diameter of from about 0.05 to about 1 micron in water; polymerizing the resulting suspension by heating; subsequently optionally washing and drying the polymer product; and subsequently mixing and heating said core and said polymer product wherein said polymer product forms a coating on said core, and wherein said polymer possesses an average particle diameter in the range of about 0.05 to about 1 micron.

2. A process in accordance with claim 1 wherein the A block of AB type block copolymer component is selected from the group consisting of  $\alpha$ -methyl-styrene, p-chlorosty-

## 16

rene; vinyl ketones; vinyl naphthalene; unsaturated monoolefins; vinylidene halides; fluorinated vinyl compounds, methyl acrylate, ethyl acrylate, butyl acrylate, dodecyl acrylate, octyl acrylate, phenyl acrylate, methyl methacrylate, ethyl methacrylate, butyl methacrylate, octyl methacrylate, monobutyl maleate, dibutyl maleate; vinyl chloride, vinyl benzoate; vinylidene chloride; pentafluoro styrene and allyl pentafluorobenzene; and the monomer forming the B block of the AB type block copolymer component is selected from the group consisting of acrylic acids, methacrylic acids, acrylamide, acrylonitrile, ethylene oxide, N-vinyl pyrrolidinone, maleic acid, vinylsulfonic acid, styrenesulfonic acid, 2-acrylamido-2-methylpropanesulfonic acid, 3-vinylxylopropane-1-sulfonic acid, 2-methacryloyoxy ethanesulfonate, 3-methacryloyoxy-2-hydroxypropanesulfonate, 2-acrylamido-2-methyl propanesulfonate, 3-sulfo-2-hydroxypropyl methacrylate, vinylphosphonic acid, 4-vinylphenol, N-vinylsuccinimide; diallyldimethylammonium chloride, diallyldiethylammonium chloride, diethylaminoethyl methacrylate, dimethylaminoethyl methacrylate, methacryloyoxyethyl trimethylammonium sulfate methacryloyoxyethyl trimethylammonium chloride, and 3-(methacrylamido)propyltrimethylammonium chloride.

3. A process in accordance with claim 1 wherein the AB type block copolymer is a copolymer of polystyrene-b-polyacrylic acid.

4. A process in accordance with claim 1 wherein the AB copolymer is a copolymer of polystyrene-b-polyoxyethylene or polystyrene-b-polymethyl methacrylate.

5. A process in accordance with claim 1 wherein said AB block copolymer possesses a number average molecular weight of from about 5,000 to about 50,000, and a weight average molecular weight of from about 10,000 to about 2,000,000, and the conductivity of said polymer coating is from about  $10^{-10}$  (ohm-cm) $^{-1}$  to about  $10^{-4}$  (ohm-cm) $^{-1}$ .

\* \* \* \* \*